

# United States Patent [19]

Akiyama et al.

[11] 3,894,142

[45] July 8, 1975

[54] **METHOD FOR PRODUCING GADOLINIUM MOLYBDATE SINGLE CRYSTALS HAVING HIGH TRANSPARENCY**

3,647,697 3/1972 Ballman et al. .... 23/301 SP  
3,773,898 11/1973 Aizu et al. .... 423/593 X

[75] Inventors: **Seikichi Akiyama, Kokubunji, Tokyo; Hirotugu Kozuka, Tokyo, both of Japan**

Primary Examiner—Herbert T. Carter  
Attorney, Agent, or Firm—Craig & Antonelli

[73] Assignee: **Hitachi, Ltd., Japan**

[22] Filed: **July 28, 1972**

[21] Appl. No.: **276,166**

[52] U.S. Cl. .... **423/263; 23/301 SP; 23/305; 423/593**

[51] Int. Cl. .... **C01g 39/00; C01g 57/00**

[58] Field of Search .... **423/263, 593; 23/301 SP, 23/304, 305**

## [56] References Cited

### UNITED STATES PATENTS

3,437,432 4/1969 Borchardt ..... 423/263

[57]

## ABSTRACT

A method for producing gadolinium molybdate single crystals is particularly characterized by its cooling step wherein when passing through a temperature zone of at least 900°C. to 700°C., the molybdate material is cooled at a cooling rate of at least 200°C./hr. According to this method there is obtained gadolinium molybdate single crystals with excellent transparency that is as high as 70 to 82% in light permeability at 6,328 Å wavelength. The obtained single crystals are of high utility value and can be most advantageously used for various types of optical materials.

**4 Claims, 2 Drawing Figures**



FIG. 1



FIG. 2



**METHOD FOR PRODUCING GADOLINIUM  
MOLYBDATE SINGLE CRYSTALS HAVING HIGH  
TRANSPARENCY**

**BACKGROUND OF THE INVENTION**

This invention relates to a method for producing gadolinium molybdate ( $Ga_2(MoO_4)_3$ ) single crystals having high transparency.

Gadolinium molybdate single crystals are generally ferroelectric and ferroelastic and also light-penetratable. Consequently, these crystals provide very excellent characteristics when used as optical material.

Although these single crystals have many excellent physical properties for use as optical materials as noted above, one problem in manufacturing such crystals is that it is extremely difficult to obtain high quality crystals. This problem is hereinafter discussed in greater detail.

It is well known that in order to obtain gadolinium molybdate crystals of good quality by using the technique of growing single crystals from the melt of high temperature according to a pull method (which is generally known as "Czochralski method"), it is usually necessary 3, the speed at which the single crystal is pulled up onto the melt surface and to also lower the cooling rate. The former step (to reduce the pull-up speed) is envisaged to minimize the crystal imperfections and separation of impurities, while the latter step (to reduce the cooling rate) is designed to preclude occurrence of cracks in the crystals due to heat distortion and internal stress strain. Usually, these single crystals are produced in the following way: first, gadolinium oxide and molybdenum oxide are mixed in the form of powder at a mol ratio of 1 : 3, then the mixture is fired at a temperature of around 1,000°C., the fired product being then melted and a seed crystal is immersed in the melt and rotated to raise up a single crystal according to the pull method. After the crystal has grown to a certain extent, it is pulled up from the melt and immediately subjected to slow cooling.

In these single crystals, a sharp crystal deformation takes place at around the Curie temperature (i.e. 45 160°C.) to give rise to a large strain stress. Consequently, cracks are very liable to occur during the cooling step in the course of crystal growth, and in some cases, the entire crystal may be even broken into pieces. It is therefore important for obtaining good quality crystals to reduce the cooling speed as much as practical. It is also necessary to extremely lower the crystal growing speed because the crystals are of a polymolecular structure where two different oxides, i.e. gadolinium oxide and molybdenum oxide, are compounded and also because the mixing rate of these two oxides must be stoichiometrically satisfied. If the single crystal growing is conducted with due consideration given to the above-said properties of gadolinium molybdate crystals, there can be obtained single crystals which are free of cracks and have a stoichiometrical mixing rate. However, these single crystals are mostly unsatisfactory in transparency, with their light penetrability or permeability being usually within the range of 30 to 50%. Such poor penetrability causes the scattering of light chiefly at the fine granular white points lying sporadically in the crystal structure.

**SUMMARY OF THE INVENTION**

An object of the present invention is to obtain gadolinium molybdate single crystals having high penetrability. According to the present invention, there is provided an improved method for producing gadolinium molybdate single crystals having as high as 70 to 82% light penetrability. This method is particularly characterized by its cooling step in which (as hereinafter described in greater detail) the work mixture is cooled at a specific cooling rate while passing through a specific temperature zone. The single crystal producing method according to the present invention comprises essentially: the step of heating and melting a polycrystal of 10 gadolinium molybdate ( $Gd_2(MoO_4)_3$ ) or heating an admixture of molybdenum oxide and gadolinium oxide 15 blended to meet a stoichiometrical value for forming said gadolinium molybdate, at a temperature higher than the melting point of said admixture to form a melt; 20 the steps of immersing a seed crystal in said melt, and 25 growing a single crystal of gadolinium molybdate according to a pull method (Czochralski method); and the step of cooling said single crystal, said cooling being carried out at a rate of higher than 200°C./hr while passing through the temperature zone of at least 900°C. to 700°C. during said cooling step.

Thus, it will be understood that the present invention is based on the finding of the inventors that the cooling rate in the cooling step after the growth of crystal, particularly the cooling rate in the temperature zone of from 900°C. to 700°C., exerts a decisive influence to light penetrability of the final crystal product.

**BRIEF DESCRIPTION OF THE DRAWINGS**

35 FIG. 1 diagrammatically illustrates one embodiment of the present invention, showing a light penetrability curve of the single crystal as observed when the cooling rate in the cooling step after pulling up the single crystal is varied; and

40 FIG. 2 is a characteristic curve showing variation of the light penetrability as a single crystal of 35% penetrability is subjected to heat treatment at various temperatures.

**DESCRIPTION OF THE PREFERRED  
EMBODIMENTS**

The invention will be further understood from the following typical example.

**EXAMPLE**

55 Gadolinium oxide and molybdenum oxide, both in the form of powder, were mixed at the mol ratio of 1 : 3 and well pulverized and mixed up. The powder mixture was then shaped into a small flat plate-like mass and fired in the air at 700°C. for 4 hours. The fired product was again pulverized into powder, which was then well mixed and again shaped into a small flat plate-like mass, the formed mass being fired in the air at 1000°C. for about 4 hours. The fired product thus obtained was then packed in a crucible and melted by heating at 1,170°C. in the air. Then, a seed crystal was fixed to a platinum support and the (001) face of said crystal was immersed in said melt, and then said support was gradually pulled up at a speed of about 8 60 mm/hr while rotating it at a speed of about 120 r.p.m., whereby a columnar gadolinium molybdate single crystal measuring 15 mm in diameter and 50 mm in length 65

was grown. The obtained crystal was cut off from the melt and the crystal temperature was maintained at the range of 1,020° to 970°C. Then, the crystal was cooled from this range of temperature down to a temperature close to the Curie point (160°C.) at various cooling rates shown on the abscissa of the graph shown in FIG. 1. Light penetrability of the thus obtained specimens was measured to obtain a result expressed by the cooling rate-penetrability curve in FIG. 1. Measurement of penetrability was made by using a He-Ne laser (output 15 mW, wavelength 6,328 Å) as light source.

As apparent from the figure, light penetrability is greatly influenced by the cooling rate. Usually, penetrability or permeability of over 60 to 70% level is required for an optical material to be servable in practical use. According to the present invention, as apparent from the curve of FIG. 1, it is possible to obtain an excellent crystal having penetrability of over 70% by selecting a cooling rate of higher than 200°C./hr. If a cooling rate of higher than 450°C./hr is used in the present invention, there can be obtained a crystal having splendid penetrability of as high as 82% which is close to the theoretical penetrability.

As obvious from the cooling rate penetrability curve heretofore described, the light penetrability of the crystals obtained at a cooling rate of higher than 450°C./hr is substantially equal to the theoretical penetrability (82%). As the results of experiments, it has been found possible to obtain a crystal having very excellent light penetrability, with no trace of cracks being created even at an extraordinarily high cooling rate of from 3,000° to 6,000°C./hr (50° to 100°C./mm). However, merely increasing the cooling rate above certain limits ends up with bad economy, so the most practical range of cooling rate is, in most cases, within the range of from 200°C. to 1,500°C./hr.

As is also evident from the curve shown in FIG. 1, a cooling rate on the order of 150°C./hr or higher is sufficient to obtain a crystal with light penetrability of 60% or higher.

In the foregoing example, air was employed as the crystal growing atmosphere, but in the present invention, any other oxidizing atmosphere containing oxygen can be used. Also, the rotational speed of the seed crystal is not limited to 120 r.p.m. as in the above example, but can be suitably selected from the range of 50 to 180 r.p.m. Further, the crystal pulling-up speed is not restricted to 8 mm/hr but is selectable from the range of 1 to 50 mm/hr. Thus, it will be understood that, in the present invention, the ordinary conditions for producing a crystal by the pulling method can be used until the point where the crystal growth is completed and that the characteristic feature of the invention resides in the

cooling step which is practiced after completion of the crystal growth.

FIG. 2 shows a heating temperature-penetrability curve which further shows how light penetrability (i.e. 5 penetrating power) varies when a gadolinium molybdate single crystal of 35% light penetrability at normal temperature (obtained by a known method) is heated gradually to higher temperatures. It is learned from this 10 curve that the temperature zone in which the crystal is apt to become non-transparent is between 700°C. and 900°C. This means that, in the cooling step in the production of single crystals, it is essential to minimize the period in which the crystal is left exposed to the temperature range of from 900°C. to 700°C. For this 15 reason, it is required in the present invention to perform the cooling at a cooling speed of over 200°C./hr in the temperature zone of 900°C. to 700°C.

As will be appreciated from the foregoing explanation, it is possible with the present invention to obtain 20 excellent gadolinium molybdate single crystals having light penetrability which is higher than at least 70%. Thus, the present invention realizes an amazing enhancement of utility value of said crystals for use as optical materials and greatly contributes to the benefit of 25 the industries concerned.

While the novel principles of the invention have been 30 described, it will be understood that various omissions, modifications and changes in these principles may be made by one skilled in the art without departing from the spirit and scope of the invention.

What is claimed is:

1. In a method for producing gadolinium molybdate 35 single crystals wherein a polycrystal of gadolinium molybdate or a mixture of molybdenum oxide and gadolinium oxide blended at such a rate as to meet the stoichiometric value for forming gadolinium molybdate is heated and melted, a seed crystal is immersed in said melt and a single crystal of gadolinium molybdate is 40 grown according to the pull method, and the resulting single crystal is cooled; the improvement which comprises the cooling of said crystal during the cooling step in the temperature zone of at least 900°C. to 700°C. at a cooling rate of over 200°C./hr.

2. The method according to claim 1, wherein said cooling is conducted under an oxygen-containing atmosphere.

3. A method according to claim 1, wherein the cooling in the temperature zone of at least 900°C. to 700°C. 50 is performed at a cooling rate of 200°C. to 1,500°C./hr.

4. The method according to claim 1, wherein the cooling rate is about 450°C per hour or higher.

\* \* \* \* \*